

No. 805,475.

PATENTED NOV. 28, 1905.

W. E. LAYCOCK.

MATERIAL FOR APPLYING OIL TO AXLE BEARINGS.

APPLICATION FILED NOV. 17, 1904.

FIG. 1.



FIG. 2.



FIG. 3.



FIG. 4.



INVENTOR:

William Ernest Laycock,  
By Attorneys,

Arthur G. Fraser & Co.

WITNESSES:

Fred White

Renf Brune

# UNITED STATES PATENT OFFICE.

WILLIAM ERNEST LAYCOCK, OF SHEFFIELD, ENGLAND.

## MATERIAL FOR APPLYING OIL TO AXLE-BEARINGS.

No. 805,475.

Specification of Letters Patent.

Patented Nov. 28, 1905.

Application filed November 17, 1904. Serial No. 233,054.

*To all whom it may concern:*

Be it known that I, WILLIAM ERNEST LAYCOCK, a subject of the King of Great Britain, residing at Sheffield, England, have invented 5 certain new and useful Improvements in the Manufacture of Material for Applying Oil to Axle-Bearings, of which the following is a specification.

This invention relates to a new product for use in the filling of journal-boxes or in other positions where a lubricant is to be applied, and to a process of preparing such an improved filling. The material generally in use at present for this purpose is cotton-waste, and this quickly loses its springiness and sinks, and thus fails to effect the intended object, which is to raise the lubricant by capillary action and apply it to the axle. This failure is a common cause of axles becoming overheated. 20 The present invention provides a combination of elastic fibers—such, for example, as horsehair or other hair with fibers of absorbent material—such, for example, as woolen threads or waste, the two being spun together and the elastic fibers being preferably given a permanent curly set and the mass being then carded or teased into a loose open condition. The elastic fibers constitute a substantially permanent elastic medium which prevents the 25 mass from sinking and packing and keeps it in constant contact with the axle, the woolen or other absorbent fibers serving to carry the oil up from the box by capillary action. The curled elastic medium is thoroughly intermingled with the absorbent medium, so as to 30 make the entire mass homogeneously elastic.

The accompanying drawings illustrate the manufacture of the improved filling, being chiefly diagrammatic. 40 Figure 1 illustrates the successive steps of forming the curl. Fig. 2 illustrates the soaking of the curl, and Fig. 3 the drying of the curl. Fig. 4 illustrates the commercial product and the manner of using it.

45 Referring to the drawings, threads of wool or the like are indicated at A and threads of horsehair or the like at B. A suitably-proportioned number of these hairs are carded together in order to effectually mix the two 50 materials without damaging the wool, and by any usual or suitable means, such as are com-

mon in spinning machinery, are then twisted tightly together to form a sort of rope C and then crimped into a kinky curl D, so that when opened out for use they assume the appearance of a loose open mass of spirals. Suitable lengths of this curl are then soaked in water, as indicated in Fig. 2, which softens the hair in its spun position. Thereupon the curl is taken out of the water and put into an oven or other drying apparatus, which is indicated in Fig. 3 with a gas-heater underneath for the sake of illustration. When dried, the hair will be found to have a permanent set in its spun and curled position. These curls of material are preferably the form of the product in which it is marketed. They are very compact and make the handling and transportation of the product simple and cheap. In use the end of the curl will be untwisted 60 to what is termed the "soft" curl and teased or carded in the manner indicated at E to form an open loose bulk such as is required to be put into the journal-boxes, and where customers have not conveniently the means 65 of teasing or carding it I propose to market it in the open loose condition indicated at E.

Though I have described with great particularity of detail certain embodiments of the invention, yet it is not to be understood 70 therefrom that the invention is limited to the specific embodiments disclosed.

Various modifications may be made by those skilled in the art without departure from the 75 invention.

What I claim is—

1. The improved material for applying oil to axle-bearings, consisting of elastic fibers and fibers of absorbent material spun together.
2. The improved material for applying oil to axle-bearings, consisting of elastic hair and fibers of absorbent material spun together.
3. The improved material for applying oil to axle-bearings, consisting of elastic fibers and fibers of absorbent material spun together, 95 in a compact curl.
4. The improved material for applying oil to axle-bearings, consisting of elastic fibers and fibers of absorbent material spun together, the elastic fibers having a permanent set in 100 their spun position.
5. In the process of manufacturing a mate-

rial for applying oil to axle-bearings, the spinning of elastic fibers and fibers of absorbent material together, soaking the product to soften the elastic fibers, and then drying the 5 product to give the elastic fibers a permanent set in their spun position.

In witness whereof I have hereunto signed

my name in the presence of two subscribing witnesses.

WILLIAM ERNEST LAYCOCK.

Witnesses:

DOMINGO A. USINA,  
FRED WHITE.